

# United States Patent

Kiyohara et al.

[15] 3,668,085

[45] June 6, 1972

[54] **METHOD OF ELECTROLYTICALLY COATING LEAD DIOXIDE ON THE SURFACE OF VARIOUS MATERIALS**

[72] Inventors: **Shinzo Kiyohara; Yasuichi Shibasaki**, both of Yokohama, Japan

[73] Assignee: **Isomura Sangyo Kaisha, Ltd.**, Tokyo, Japan

[22] Filed: **Aug. 21, 1969**

[21] Appl. No.: **852,074**

[30] **Foreign Application Priority Data**

Aug. 24, 1968 Japan.....43/60211

[52] U.S. Cl.....204/57

[51] Int. Cl. ....C23b 11/00

[58] Field of Search.....204/57

[56]

## References Cited

### UNITED STATES PATENTS

3,463,707 8/1969 Gibson et al.....204/57  
3,213,004 10/1965 Schmidt.....204/57

*Primary Examiner*—John H. Mack

*Assistant Examiner*—R. L. Andrews

*Attorney*—Sughrue, Rothwell, Mion, Zinn & Macpeak

[57]

## ABSTRACT

Lead dioxide is coated on the surface of a base electrode by electrolyzing an acidic aqueous lead nitrate solution containing a small amount of copper nitrate at a temperature not lower than 70° C. and with a current density of anode not higher than 4 A/dm<sup>2</sup>.

**2 Claims, No Drawings**

**METHOD OF ELECTROLYTICALLY COATING LEAD DIOXIDE ON THE SURFACE OF VARIOUS MATERIALS**

The present invention relates to a method of galvanizing electrolytically lead dioxide coating on the surface of a base electrode consisting of various materials.

It is well known that a lead dioxide electrode having originally a high oxygen over voltage and hardly soluble characteristics in electrolytic solution has failed to be useful industrially due to its insufficient mechanical strength of the deposited or plated lead dioxide even though lead dioxide itself is a hard and brittle material, and due to the difficulties encountered for the manufacturing of large lead dioxide electrode in such a commercial size as is normally used by an artificially made graphite electrode in the electro-chemical industry.

It is also a well known matter that a number of experiments have been carried out to deposit or galvanize electrolytically a lead dioxide coating on the surface of some base electrode, such as a tantalum-, or a nickel-screen, or on the surface of a graphite base electrode to improve the difficulties stipulated to enlarge lead dioxide electrode itself in the foregoing paragraph.

However, the inventors are of the opinion from their experiments that the life of a thus electrolytically deposited or plated lead dioxide coating on a certain base electrode in an acidic lead nitrate solution is greatly dependent upon the conditions under which the electrolysis is carried out.

Namely, due to complicated factors under which the electrolytic plating or coating is made on the surface of base electrode, for instance, such as the difference in the material of the base electrode and that of the electrolytic conditions used in the deposition of lead dioxide, the development of a coating having the excellent characteristic of difficult solubility in a salt solution and having a high over voltage for oxygen, has been unsuccessful.

The inventors have recently found and confirmed by X-ray diffraction analysis of the layer of lead dioxide coating that one of the reasons for the decay or cleavage of this coating is attributable to the transition of amorphous lead dioxide electrolytically deposited into crystalline lead dioxides during the course of the applied electrolysis after the coating was prepared.

The present invention relates to the establishment of optimum electrolytic conditions under which a durable lead dioxide coating or plating can be made on the surface of a base electrode.

A detailed explanation of the conditions will be given in the following paragraphs:

An artificial graphite electrode as an anode of an electrolytic cell for the electrolysis of an alkali-chloride solution in the chlorine industry is the only available material for commercial use. However, the quality of the graphite itself is directly related to the current efficiency, the operating life of the cell, and to the purity of the produced chlorine gas.

As the electrode distance between the anode and the cathode is normally fixed by the structural characteristics of the electrolytic cell, any decay of the active surface of the graphite anode in the course of the progressing electrolysis will tend to increase the distance to the opposite cathode and it will cause a decrease in current efficiency of the cell and an increase in power consumption per unit amount of chlorine. Frequent lowering of the anode will be necessary and the replacement of decayed anodes will appreciably decrease the operating efficiency of the factory.

Especially in case of sodium chloride electrolysis using a mercury cathode, the graphite anode will decay and drop physically due to the porosity and the graphite powder disintegrates the sodium amalgam to produce gaseous hydrogen and it is mixed in the chlorine gas. This is one of the reasons an explosive gas mixture of hydrogen and chlorine can be obtained.

A platinum anode is preferable for such an anode having the nature of only a slight solubility in a salt solution and having a

high oxygen over voltage, but it is too expensive due to the shortage of supply, thus the application of platinum anode is limited to the anode for a high grade of oxidation in the production of perchlorate, periodate, and persulphate which needs an extremely high oxygen over voltage.

Although the oxygen over voltage is a little lower than platinum, a lead dioxide anode is favored due to its abundance and easiness to produce by the electrolysis of a lead salt solution, and it has a reasonably difficult solubility comparable with platinum.

Electrolytically deposited lead dioxide is resistant to halogen ions, nitrate ion, and sulphate ion, and therefore it is quite suitable as an anode for the electrolysis of these salt solutions. By the application of a lead dioxide anode, the adjustment of the distance between the anode and the cathode of the cell will become negligible and it will contribute to getting higher current efficiency as well as higher productivity of the cell. Especially, the merit of using a lead dioxide anode can be

found in getting pure chlorine gas from the anode, because a graphite anode will give carbon dioxide inevitably mixed with chlorine gas together with a mixing of hydrogen due to the catalytic disintegration of sodium amalgam by the dropping powder of graphite, as was already mentioned in the foregoing paragraph.

It was already reported in Journal Electro-Chemical Soc. Japan 552 (1959) 27, that electrolytically deposited lead dioxide had three configurations of amorphous, crystalline alpha-type (rhombic system), and beta-type (tetragonal system), while lead dioxide made from acidic lead nitrate solution consists of alpha- and beta-type lead dioxide as a mixture, but lead dioxide deposited from alkaline lead salt solution contains alpha-type lead dioxide only. However, no information has been available to explain the mixing rate of these three configurations as well as the producing conditions for the respective types of lead dioxide by electrolysis.

The inventors tried for the first time to check this matter by a phase analysis using an X-ray defraction method for the deposited lead dioxide which was prepared under following conditions:

|                                       |                                                                                                                               |
|---------------------------------------|-------------------------------------------------------------------------------------------------------------------------------|
| Electrolytic cell:                    | as reported in Journal Electro-Chemical Soc. Japan 59 (1968) 36                                                               |
| Electrolytic solution:                | Pb(NO <sub>3</sub> ) <sub>2</sub> mol/liter, Cu(NO <sub>3</sub> ) <sub>2</sub> 0.1 mol/liter pH = 4.2                         |
| Bath temperature:                     | 30°-70° C                                                                                                                     |
| Current density:                      | 1-10 A/dm <sup>2</sup> at the anode                                                                                           |
| Base metal of anode:                  | Platinum plate                                                                                                                |
| Lead dioxide used in the experiments: | Electrolytically deposited lead dioxide on platinum plate is taken off, and it was washed with distilled water and was dried. |

Following results were found:

1. Content of alpha lead dioxide is larger at a higher temperature of the electrolytic bath, however, no appreciable difference was found in the temperature range of 50° - 70° C. A higher current density will give a lower content of alpha lead dioxide.

2. Generally speaking, a higher content of beta lead dioxide is obtained the higher the temperature of electrolysis, except in the case the electrolysis temperature is low and the current density is also low.

At a lower temperature, the variation of the content of beta lead dioxide is not remarkable.

3. The content of amorphous lead dioxide is higher when the bath temperature is low and the current density is high. By life tests for the electrolysis of a halide solution by using electrodes coated with lead dioxide until some remarkable decay or cracking of the coated layer was noticed, the following results are reported:

a. An electrode coated with lead dioxide at a lower temperature and at a higher current density during deposition had a life of 1 - 6 months of continuous use.

b. An electrode coated with lead dioxide at a higher temperature and at a lower current density during deposition had a comparatively longer life.

This will indicate that amorphous lead dioxide tends to change its configuration into crystalline forms during the period of electrolysis in the halide solution and the cleavage or decay is attributable to the change of the specific volume between these configurations. (refer to (3) of foregoing paragraph). As the result, it is quite evident that the determination of conditions under which a lesser content of an amorphous lead diox-

5 Anode:

100 mm from the top of No. 1 –  
No. 4 electrodes shown in  
Table 1 kept in the solution.  
Current density at the anode is  
3 A/dm<sup>2</sup>.

Weight Loss:

Upper part of the electrode  
above the solution is covered  
by plasticized PVC tubing.  
By decreased weight after the  
tests.

10 The results of the tests are given in Table 2.

TABLE 2

| Number | Weight of electrode |                  | Decreased weight in g. | Current used, A/dm <sup>2</sup> | Weight loss per A/dm <sup>2</sup> in mg./A/dm <sup>2</sup> | Remarks          |
|--------|---------------------|------------------|------------------------|---------------------------------|------------------------------------------------------------|------------------|
|        | Before test in g.   | After test in g. |                        |                                 |                                                            |                  |
| 1      | 137.9263            | 137.7370         | 0.1873                 | 356                             | 0.525                                                      | Pin holes found. |
| 2      | 140.6917            | 140.5835         | 0.1082                 | 485                             | 0.223                                                      | Crackings found. |
| 3      | 139.4512            | 139.4113         | 0.0399                 | 503                             | 0.0793                                                     | Few pin holes.   |
| 4      | 140.9234            | 140.9232         | 0.0002                 | 512                             | 0.000                                                      | No defects.      |

ide containing coating can be made, is the most important matter. For instance, lead dioxide coating made with a current density of 1 A/dm<sup>2</sup> at the anode and at a bath temperature of 70° C. showed a minimum content of amorphous lead dioxide in the coating. It was already reported by the inventors in Journal Electro-Chemical Soc. Japan 911 (1962) 30 that a 0.5 – 1.35 mm thickness of a lead dioxide coating could be made at a 30° – 65° C. bath temperature, 4.6 – 7.0 A/dm<sup>2</sup> current density at the anode from an acidic lead nitrate solution upon the surface of carbon or graphite base electrode.

Thus, the present invention is characterized in that an aqueous solution of acidic lead nitrate is electrolyzed by using a bath temperature higher than 70° C. and a current density lower than 4 A/dm<sup>2</sup> in order to minimize the content of amorphous lead dioxide.

#### EXAMPLE 1

The base electrode used in this experiment was made in accordance to the process described in Japanese Pat. No. 450,342 or U.S. Pat. Nos. 3,434,905 and 3,318,794 by the inventors, which consists of a center copper bar of 3 mm in diameter and 210 mm in length, and silver is galvanized on its surface upon which lead dioxide powder mixed with a thermoplastic resin was hot-pressed to make a lead dioxide base electrode having a diameter of 8 mm and a coating length of 180 mm with a semi-spherical end piece.

The thus prepared base electrode now underwent another process for the electrolytic deposition of lead dioxide by using it as anode and a copper bar as cathode in an acidic lead nitrate solution under constant current density and other conditions given in Table 1.

TABLE 1

| Number | Electrolyte                                |                                            |     | Conditions of electrolysis |                                             |            |                                              |                                              |
|--------|--------------------------------------------|--------------------------------------------|-----|----------------------------|---------------------------------------------|------------|----------------------------------------------|----------------------------------------------|
|        | Pb(NO <sub>3</sub> ) <sub>2</sub> , mol/l. | Cu(NO <sub>3</sub> ) <sub>2</sub> , mol/l. | pH  | Sp. gr.                    | Current density at anode, A/dm <sup>2</sup> | Temp., °C. | Thickness of PbO <sub>2</sub> deposited, mm. | Spec. resistance × 10 <sup>4</sup> , ohm-cm. |
| 1      | 1.08                                       | 0.17                                       | 4.2 | 1.32/20° C.                | 4.5                                         | 22±1.5     | 1.15                                         | 7.5                                          |
| 2      | 1.08                                       | 0.17                                       | 4.2 | 1.32/20° C.                | 4.0                                         | 25±2       | 1.85                                         | 8.0                                          |
| 3      | 1.05                                       | 0.15                                       | 4.0 | 1.28/25° C.                | 5.0                                         | 70±2       | 1.75                                         | 5.3                                          |
| 4      | 1.05                                       | 0.15                                       | 4.0 | 1.28/25° C.                | 3.5                                         | 77±2       | 1.80                                         | 3.9                                          |

The thus coated lead dioxide layers can only be checked the the stability by using it in a practical manner in the electrolysis of salt solutions. The inventors employed following process to check the life of the coatings in a comparatively short period.

Electrolytic solution: 0.2 mol/l KH<sub>2</sub>PO<sub>4</sub> 50 ml, 0.2 mol/l NaOH 43 ml pH = 7.6  
Bath temperature: 40° ± 2° C.  
Current: 1 ampere  
Period of tests: 3 weeks  
Vessel: 80 mm in diameter, 210 mm in length, normal steel jar as cathode

4 Anode:

100 mm from the top of No. 1 –  
No. 4 electrodes shown in  
Table 1 kept in the solution.  
Current density at the anode is  
3 A/dm<sup>2</sup>.

Weight Loss:

Upper part of the electrode  
above the solution is covered  
by plasticized PVC tubing.  
By decreased weight after the  
tests.

#### EXAMPLE 2

According to Japanese Pat. Nos. 450,342 and 466,747, by the inventors, hollow units having an outer diameter of 48 mm, an inner diameter of 34 mm and a length of 100 mm obtained by molding electrolyzed lead dioxide containing a small amount of a thermoplastic synthetic resin as an adhesive in a sealed pressure proof mold under pressure and at elevated temperature were connected under pressure and at elevated temperature to 730 mm including a semi-spherical end piece. The inside of this electrode was washed with water and was electrolytically galvanized with a silver coating of 10 microns in thickness by a known process. Again it was washed with water and was galvanized with a copper coating of 20 microns from an acidic copper sulphate solution. The outside surface of this base electrode was covered still with a film of thermoplastic resin during hot-press processing, it was mechanically removed and cleaned to remove resinous material with some solvents. The treated outside surface of the base electrode now underwent the lead dioxide coating process by the following:

Electrolyte: Pb(NO<sub>3</sub>)<sub>2</sub> 1 mol/l, Cu(NO<sub>3</sub>)<sub>2</sub> 0.1 mol/l pH = 3.5–3.7  
Bath temperature: 70° ± 2° C.  
Current density: 3 A/dm<sup>2</sup> at the anode  
Thickness of PbO<sub>2</sub> coating: 2 mm

The 6 electrodes thus prepared were tested in a commercial electrolytic bath using a 500 ampere cell without the use of a diaphragm to produce sodium chloride by the electrolysis of a saturated sodium chloride solution to which 3 g/l of sodium chromate was added at pH of 6.7 – 6.85. The current density

5 at the lead dioxide anode was 12.3 – 13.8 A/dm<sup>2</sup>, a bath voltage of 3.7 – 3.9 volt with a continuous and total power supply of 8,250 KWH.

65 All of these electrodes showed no defect after the electrolysis and no lead ion was identified in the solution after the electrolysis and the color of solution on completion was a thin yellow and clear.

70 The present industrial process to make sodium chlorate uses a graphite anode which is liable to give a dark mother solution after the electrolysis due to decayed carbon powder coming from the anode, and it will take expensive and big installations to get a clear mother solution as well as higher labor costs to recover pure end products.

This invention seems to give a reliable and reasonable process for the electrolytic production of various useful materials on an industrial scale.

What is claimed is:

1. In a method of electrodeposition of a coating of lead dioxide on the surface of a base electrode which comprises electrolyzing an acidic lead nitrate solution containing a small amount of copper nitrate, the improvement which comprises

maximizing the quantity of lead dioxide in the beta configuration, the amount of copper nitrate in said solution ranging from 0.1 to 0.17 mol/liter, the amount of lead nitrate in said solution ranging from 1 to 1.08 mol/liter, the temperature of said solution ranging from 70° to 100° C. and the current density at the anode ranging from 1 to 4 A/dm<sup>2</sup>.

2. The method of claim 1, wherein the current density at the anode ranges from 3 to 4 A/dm<sup>2</sup>.

\* \* \* \* \*

10

15

20

25

30

35

40

45

50

55

60

65

70

75